

## UNITED STATES PATENT OFFICE

2,211,872

## TREATMENT OF TEXTILE MATERIALS

Alexander James Wesson and George Holland  
Ellis, Spondon, near Derby, England, assignors  
to Celanese Corporation of America, a corpora-  
tion of Delaware

No Drawing. Application August 5, 1938, Serial  
No. 223,218. In Great Britain September 9,  
1937

7 Claims. (Cl. 8—124)

This invention relates to the treatment of textile materials comprising filaments, yarns, ribbons or the like of cellulose or regenerated cellulose and especially high tenacity filaments, yarns, ribbons and the like of regenerated cellulose.

By swelling regenerated cellulose textile materials, and particularly regenerated cellulose textile materials formed by saponification of textile materials having a basis of cellulose acetate or other cellulose esters, e. g. stretched cellulose ester materials which have been saponified with solutions of caustic soda or other strong alkalies, the affinity of the materials for cotton dyestuffs can be enhanced and the serimetric properties, e. g. flexibility and extensibility, can be improved.

We have now found that particularly valuable results may be obtained in this process, and any tendency of the treating solution to act deleteriously on the regenerated cellulose may be reduced, if the materials are treated with solutions of caustic soda or other strong alkali which contain compounds capable of acting as buffers in alkaline solution. The process has the additional very considerable advantage that it is possible by means of it to treat textile materials which contain both regenerated cellulose and cellulose esters so as to enhance the affinity of the regenerated cellulose for dyestuffs without causing any substantial saponification of the cellulose esters. Fabrics which contain both yarns of regenerated cellulose and yarns of cellulose esters are of considerable commercial importance from the point of view of obtaining differential dyeing effects, as, for example, when the fabric is dyed with a dyestuff which has an affinity only for the regenerated cellulose yarns leaving the cellulose ester yarns white. It is, therefore, of considerable importance to be able to improve the affinity of the regenerated cellulose yarns for the dyestuffs without at the same time deleteriously affecting the resist properties of the cellulose ester yarns.

The strong alkali employed may be caustic soda, as indicated above, or it may be lithium hydroxide, caustic potash or a quaternary ammonium compound such as trimethyl benzyl ammonium hydroxide.

Particularly satisfactory results have been obtained by the use of sugars as the buffering compounds and it is, therefore, preferred to use these bodies. Various sugars may be used, for example, cane sugar or other di-oses or poly-oses. Particularly good results have been obtained with the aid of glucose, dextrose, laevulose, galactose and other mono-oses, and there may be employed crude products containing these sugars, for ex-

ample, the mixture of glucose and laevulose obtainable by hydrolysing cane sugar or a crude sugar containing the mixture obtainable by the hydrolysis of wood.

However, other buffering compounds may be employed, and as examples of such agents may be mentioned polyhydric alcohols, for example, mannitol, and also substances of weakly acidic character as, for example, the amino acids, e. g. the aliphatic amino acids, as, for example, glycine or the di- or poly-peptides in which two or more acid or amino residues are united, e. g. glycyl-glycine. Suitable amino acids or di- or poly-peptides are, for example, those readily obtainable by the acid or alkaline hydrolysis of proteins. Crude hydrolysis products obtainable by hydrolysing wool or other protein material with aqueous alkali may also be employed. Other substances are weak inorganic acids, e. g. boric acid, and, in general, there may be employed neutral or weakly acid substances which are capable of forming salts with alkalies.

The concentrations of the strong alkali and the buffering agent will depend largely on the nature of the materials treated and of the alkali used as well as on the temperature at which it is desired to work. In general as the temperature is reduced the action of a given concentration of alkali in increasing the dye affinity is enhanced and at the same time the danger either of deleterious action of the solution on the cellulose linkages and of saponification of cellulose ester materials present in admixture with the cellulosic materials is reduced. Low temperatures, e. g. below 10° C. or even below 5 or 0° C., e. g. down to —5° C. are therefore preferred but it is possible to work at higher temperatures, e. g. 20° C. or higher. In general, concentrations of aqueous caustic soda between 35% are most useful. Thus, valuable results are obtainable at temperatures below about 11° C. with solutions containing 5-30% of caustic soda and about 5-20% glucose and particularly useful results are obtainable by the use of solutions containing 8-12% of caustic soda and about the same amount of glucose, at temperatures below 5° C. and preferably in the neighborhood of 0° C. Lithium hydroxide can be used in similar concentrations but caustic potash must be more concentrated to get similar results and the same is true of the quaternary ammonium bases. In general, the higher the tenacity of the materials treated the less rigorous need be the conditions to get the desired results. The time of treatment is preferably very short, e. g. 1, 2 or 3 minutes but with more dilute solu-

tions than those contemplated above a longer time of treatment is permissible, though this may introduce some danger of saponifying any cellulose ester materials present.

- 5 The alkaline medium containing the buffering compound may be applied to any form of textile material, e. g. textile material in the form of yarns or other filamentary materials or in the form of fabrics, and may be applied by any suitable method, e. g. by passing the textile materials through a bath of the alkaline medium containing the buffering compound. It is desirable that the materials, immediately after being contacted with the alkaline medium for the requisite time, should be quickly washed in order to stop the action of the alkaline medium.

The following examples illustrate the invention:

*Example 1*

- 20 Regenerated cellulosic yarn made by the complete saponification of cellulose acetate yarn stretched to a considerable extent under the influence of steam is immersed for 1 minute in hank form in an aqueous bath containing 10% of caustic soda and 10% of glucose at a temperature of 0° C. An affinity for cotton dyes is imparted to the material, which, however, is not swollen to as great an extent as it would be in the absence of the glucose so that less risk of damaging the material is present.

The temperature may be maintained at 10° C. instead of 0° C. or may be between 0 and 10° C.

*Example 2*

- 35 The process is carried out as in Example 1 but employing a bath containing 30% caustic soda and 15% glucose.

*Example 3*

- 40 The process is carried out as in Example 2 but employing a solution containing 20% of caustic soda and 10% glucose.

*Example 4*

- 45 A fabric composed of regenerated cellulose of the kind used in Example 1 in admixture with cellulose acetate yarn is treated according to any of the preceding examples. In this way the affinity of the regenerated cellulose yarn 50 for cotton dyes is improved but substantial saponification of the cellulose acetate is avoided.

*Example 5*

- 55 A fabric treated according to Example 4 is dyed in a dye-bath containing 4% of Diphenyl F Scarlet 4BS and 20% of common salt, these percentages being based on the weight of the material and the bath volume being 40:1. The regenerated cellulose yarn is dyed whereas the 60 cellulose acetate yarn remains uncoloured.

In the above examples, caustic soda can be replaced by lithium hydroxide. Somewhat similar results can be obtained by employing instead of caustic soda trimethyl benzyl ammonium hydroxide in 20% concentration, the time, temperature and concentration of the glucose being the same. If caustic potash be substituted for the caustic soda, higher concentrations and/or times are required and the concentration of the glucose may be reduced. Instead of glucose may be used, for example, glycine, glycyl-glycine and sugars such as laevulose, dextrose and galactose.

In the examples, all the percentages are by 75 weight.

The invention, as indicated above, is applicable to the treatment of cellulosic textile materials generally. It is of particular importance, however, in connection with materials comprising filaments, yarns, ribbons or the like of regenerated cellulose and having a high tenacity, i. e. a tenacity higher than that obtainable by ordinary spinning processes without a spacial stretching operation. The lower limit for high tenacity yarns and the like may be taken as 10 about 1.5 grams per denier. The advantages of the present invention are best seen, however, with materials of higher tenacity than this, e. g. 1.75-2, 3, 4 or more grams per denier.

The invention has been described with particular reference to increasing the affinity of the materials for cotton dyes. The increase in affinity obtained however is accompanied by an increase in affinity for other dyes especially vat dyes in alkaline solution.

Having described our invention, what we desire to secure by Letters Patent is:

1. Process for the production of improved artificial materials which comprises treating materials containing high tenacity filaments, fibers, 25 yarns or the like of regenerated cellulose in admixture with filaments, fibers, yarns or the like of an organic ester of cellulose with a 4-35% aqueous solution of caustic soda containing 5-20% of a buffering agent at a temperature 30 below 20° C. to increase the affinity of the regenerated cellulose for cotton dyes without saponifying the cellulose ester and without deleteriously affecting the regenerated cellulose constituent.

2. Process for the production of improved artificial materials which comprises treating materials containing high tenacity filaments, fibers, 40 yarns or the like of regenerated cellulose in admixture with filaments, fibers, yarns or the like of an organic ester of cellulose with a 4-35% aqueous solution of caustic soda containing 5-20% of sugar at a temperature below 20° C. to increase the affinity of the regenerated cellulose for cotton dyes without saponifying the 45 cellulose ester and without deleteriously affecting the regenerated cellulose constituent.

3. Process for the production of improved artificial materials which comprises treating materials containing high tenacity filaments, fibers, 50 yarns or the like of regenerated cellulose in admixture with filaments, fibers, yarns or the like of cellulose acetate with a 4-35% aqueous solution of caustic soda containing 5-20% of a buffering agent at a temperature below 20° C. to increase 55 the affinity of the regenerated cellulose for cotton dyes without saponifying the cellulose acetate and without deleteriously affecting the regenerated cellulose constituent.

4. Process for the production of improved artificial materials which comprises treating materials containing high tenacity filaments, fibers, 60 yarns or the like of regenerated cellulose in admixture with filaments, fibers, yarns or the like of cellulose acetate with a 5-30% aqueous solution of caustic soda containing 5-20% of glucose at a temperature below 11° C. to increase 65 the affinity of the regenerated cellulose for cotton dyes without saponifying the cellulose acetate and without deleteriously affecting the regenerated cellulose constituent.

5. Process for the production of improved artificial materials which comprises treating materials containing filaments, fibers, yarns or the like of regenerated cellulose of tenacity at least 75

- 2 grams per denier in admixture with filaments, fibers, yarns or the like of cellulose acetate with a 5-30% aqueous solution of caustic soda containing 5-20% of glucose at a temperature below 11° C. to increase the affinity of the regenerated cellulose for cotton dyes without saponifying the cellulose acetate and without deleteriously affecting the regenerated cellulose constituent. 5
- 10 6. Process for the production of improved artificial materials which comprises treating materials containing high tenacity filaments, fibers, yarns or the like of regenerated cellulose in admixture with filaments, fibers, yarns or the like of cellulose acetate with an 8-12% aqueous solution of caustic soda containing 8-12% of glucose at a temperature below 5° C. to increase the affinity of the regenerated cellulose for cotton dyes without saponifying the cellulose acetate and without deleteriously affecting the regenerated cellulose constituents. 10 15
7. Process for the production of improved artificial materials which comprises treating materials containing filaments, fibers, yarns or the like of regenerated cellulose of tenacity at least 2 grams per denier in admixture with filaments, fibers, yarns or the like of cellulose acetate with an 8-12% aqueous solution of caustic soda containing 8-12% of glucose at a temperature below 5° C. to increase the affinity of the regenerated cellulose for cotton dyes without saponifying the cellulose acetate and without deleteriously affecting the regenerated cellulose constituents. 15

ALEXANDER JAMES WESSON.  
GEORGE HOLLAND ELLIS.